

Dec. 13, 1938.

G. F. NADEAU

2,139,767

BUFFERED PHOTOGRAPHIC FILM

Filed Feb. 15, 1936

Fig.1.



Fig.2.



Fig.3.



Fig.4.



Fig.5.



INVENTOR:

*Gale F. Nadeau,*

BY

*Newton M. Perrins  
R. Frank Smith*

ATTORNEYS.

## UNITED STATES PATENT OFFICE

2,139,767

## BUFFERED PHOTOGRAPHIC FILM

Gale F. Nadeau, Rochester, N. Y., assignor, by  
mesne assignments, to Eastman Kodak Company,  
Jersey City, N. J., a corporation of New Jersey

Application February 15, 1936, Serial No. 64,103

12 Claims. (Cl. 95—9)

This invention relates to photographic films and particularly to a method of controlling the acidity of layers coated on the film which may exert an undesirable effect on the sensitivity of the emulsion.

It is known that photographic emulsions are affected by change in acidity or hydrogen ion concentration and that a loss in speed or sensitivity results from the addition of acidic material to the emulsion. In coating a sensitive material on the film base carrying subbing or other layers designed to protect it from, or cause it to adhere to, the base, the water of the emulsion leaches materials from the sub layers or from the base. If the material leached out by the emulsion in this way has a different degree of acidity than the emulsion itself, the sensitivity of the emulsion is affected and a loss in speed or other undesirable result is produced. These 10 defects are usually manifested by lines or areas of varying sensitivity. If the acidity of the base is uniformly different from that of the emulsion, there may be an over-all loss insensitivity which becomes very bad on ageing. There may also be 15 a loss in the latent image or a loss in contrast on ageing for normal periods. When a gelatin subbing solution is applied to the film base prior to coating the sensitive emulsion, the gelatin solution may be coated at a high temperature which 20 tends to cause hydrolytic breakdown of the gelatin. This is accompanied by a drop in pH and a change in viscosity, due to the breaking down of the gelatin. As the pH drops, the accumulated acid catalyzes this hydrolytic breakdown and a 25 condition of high acidity soon results which is communicated to the sensitive emulsion later coated on the base.

It is accordingly the principal object of the present invention to provide a photographic film 40 having the acidity of the layers which come in contact with the sensitive emulsion so adjusted that the sensitive emulsion will not be adversely affected. A further object is to provide a stripping film having the acidity of the adhesive layer so adjusted that the speed and fogging 45 characteristics of the sensitive emulsion are not affected by it. A still further object is to provide a backing layer for a sensitive film which has the acidity so controlled that it will not affect 50 the sensitive emulsion when it is brought into contact with the emulsion in storage, or by rolling on a spool.

These objects are accomplished by adjusting the pH or hydrogen ion concentration of the layer 55 which may come in contact with or affect the

sensitive emulsion to the pH of the emulsion and adding to it a buffering material to maintain it substantially at that pH.

In the accompanying drawing which is by way of illustration only,

Fig. 1 represents a single view of a film having a buffered sub layer;

Fig. 2 is a sectional view of a film having a buffered undercoat between the layer and the emulsion;

Fig. 3 is a sectional view of a film having a buffered backing layer;

Fig. 4 is a sectional view of a film having emulsion layers and buffered undercoat layers on each side of the support; and

Fig. 5 is a sectional view of a stripping film having a buffered adhesive layer.

In carrying out my invention I add to the solution of the material which is to be coated on the film base, a suitable amount of a material 20 which has the required buffering action. This material may be a suitable acid salt or base salt mixture, or I may use a suitable water-soluble, non-volatile, organic acid, such as oxalic, tartaric or succinic acid, in combination with a proper 25 salt of said acid.

By "acid salt mixture" and "base salt mixture" I mean a mixture of an acid or a base with its corresponding salt, for example, citric acid and sodium citrate is an acid salt mixture, and ammonium chloride and ammonia is a base salt mixture.

It is sometimes necessary to add only an acid to buffer against an increase in acidity, the inherent buffering capacity of the gelatin taking 35 care of the buffering against an increase in alkalinity. For example, for pH ranges below about 5.5, gelatin and an added acid constitute an efficient buffer by reason of the alkaline buffering capacity of gelatin in these pH ranges.

The action of buffering materials is well recognized and will not be reviewed here. It is to be understood that I may employ any suitable buffering material in sufficient amount to obtain the desired result, it being only necessary that 45 the material be one which does not adversely affect the sensitive emulsion.

Referring to the accompanying drawing which illustrates several methods of using my invention, Fig. 1 is a view in section of a film comprising a support 10 which may be of cellulose nitrate coated with a buffered sub layer 11 and having thereon a sensitive emulsion layer 12. The buffered sub layer prevents the action of acids or other undesirable material in the base 10 from

reaching and affecting the sensitivity of the sensitive emulsion 12. In Fig. 2 the base 10 is coated with an ordinary gelatin sub layer 13 over which is coated a buffered gelatin layer 14 5 on which is laid the sensitive emulsion 12. In the base of cellulose acetate or other cellulose ester films it is frequently necessary to coat several gelatin or other layers on the film to secure adhesion of the sensitive emulsion layer, as illus- 10 trated in Fig. 2.

Fig. 3 shows a section of a film comprising the usual support 10, sub layer 13 and emulsion 12. This film has on the back thereof a gelatin layer 15 buffered to the pH of the emulsion 12 so that 15 when the film is rolled and the layer 15 comes into contact with the layer 12 the sensitivity of the layer 12 will not be affected by the materials in the layer 15 or the base 10.

Fig. 4 shows a film having an emulsion layer 12 and a buffered gelatin layer 14 on each side of a support 10. There may also be an additional sub layer 13 between the support and the buffered gelatin layer, although this layer is not essential. Other subbing layers may also be added 25 and there may be a layer over the emulsion, such as an abrasion preventing or anti-static layer.

In the photoengraving and related arts, photographic films or plates are used in which the sensitive emulsion is supported on a temporary base during exposure and formation of the image and is removed from the temporary base during processing. These emulsions are usually of a type which produces an image of extreme contrast. The emulsion is supported on a permanent base, 30 such as collodion or other cellulose derivative, which is affixed to the temporary support by means of a water-soluble adhesive. Since the emulsion has a high degree of acidity and the adhesive used to affix the permanent support 35 carrying the emulsion layer to the temporary support usually has a lower degree of acidity, stripping films previously made in this way have not been entirely satisfactory, due to the reaction between the emulsion layer and the adhesive layer, which resulted in spotting and fogging of 40 the emulsion. The permanent emulsion support, moreover, must be water permeable so that the water of the processing baths can pass through it and reach the adhesive layer. For this reason the permanent support should be one which 45 prevents reaction between the sensitive emulsion and the adhesive layer, and at the same time should be sufficiently water permeable to permit water to pass through it and reach the adhesive layer. Another requisite of the permanent emulsion support is that it should not swell or shrink 50 during or after removal from the temporary support, since this distorts the photographic image and makes it useless for its intended purpose.

A stripping film having these characteristics is illustrated in Fig. 5 in which 16 is a temporary support of paper or suitable material having a baryta coating 17. Over this is laid the adhesive layer 18 which is buffered to the pH of the sensitive emulsion. On the adhesive layer is coated the permanent support 19 of cellulose nitrate and on this is a sensitive emulsion 20, and a gelatin coating 21 is affixed to the opposite 55 side of the support 16.

The type of permanent support which I have found most suitable for the stripping film described above is one formed from a cellulose nitrate of low nitrogen content and high alcohol solubility. A cellulose nitrate of this composition

should contain approximately 9% to 12% of nitrogen. It will have a solubility in methyl alcohol of 30 to 100% and a viscosity of 2 to 5 seconds by the dropping ball method. This cellulose nitrate should be water permeable in order to 5 permit the water of the developing or other treatment baths to reach and penetrate the adhesive layer. In order to increase this water permeability it is desirable to add certain materials, such as glyceryl bori-borate, mono-, di- and tri- 10 acetin, lactic acid, glycerin, various triethanolamine derivatives, lithium chloride, lithium nitrate, cadmium bromide and other materials. The nitrate may be applied in a solution of 7½% in methyl alcohol, acetone and butyl alcohol or 15 similar solvents.

Viscosity by the dropping ball method referred to above is determined as follows: 10 grams of dry nitrocellulose is dissolved in 100 cc. of a mixture comprising 50% by volume of methyl alcohol and 50% by volume of acetone at 25° C. Viscosity is measured by the time in seconds it takes for a steel ball having a diameter of  $\frac{1}{8}$  inch and weighing .1320 gram to fall 15 centimeters through the nitro cellulose solution 25 at 25° C. in a tube having a diameter of  $1.7 \pm .05$  centimeter.

The adhesive layer may consist of glue or liquid glue or a mixture of glue and dextrin. It is also possible to coat a layer of dextrin directly 30 over the permanent support of paper or other material and to lay the glue or glue and dextrin adhesive layer buffered to the proper pH on the dextrin layer. The glue solution may be plasticized with a solvent, such as glycerin, before 35 applying it.

It is to be understood that while I have described a number of modifications of films having layers buffered according to my invention, I am not limited to films having the particular number or types of layers illustrated. Other layers 40 may also be added, as for example, a gelatin overcoating upon the emulsion to prevent abrasion of said emulsion. Additional gelatin subbing layers may be applied between the emulsion and the support or other gelatin layers may be applied over the sensitive emulsion layer or on the support. In the case of the stripping film a gelatin layer may be applied between the nitrate permanent support and the sensitive emulsion or between the nitrate permanent support and adhesive layer. The buffering backing layer may contain a dye or other material which causes it to 50 function as an anti-halation layer. The subbing layers may be composed of materials other than gelatin such as casein, agar, cellulose derivatives or resins.

The following embodiment, which is stated by way of example, is one method of forming a stripping film according to my invention.

A porous type paper coated with clay or preferably baryta is coated with a solution of glue containing glycerin. The combination of the glue solution is determined by the mode of application, the speed of coating and the temperature and viscosity of solution. With a coating speed 65 of 100 feet per hour an 18% glue containing an equal amount of glycerin is used. When dry, the cellulose nitrate dope is coated over it. This dope consists of 7½% solution of cellulose nitrate having a nitrogen content of about 12% dissolved in methyl alcohol, acetone, and butyl alcohol. This dope is coated to form a skin of about 0.0003 of an inch thick. The regular gelatin sub is applied to the nitrate skin and this is fol- 70

lowed by a sensitized silver-halide emulsion. The adhesive solution of glue is adjusted prior to coating to the hydrogen ion concentration of the emulsion by the addition of salicylic acid in the required amount, which may vary from  $\frac{1}{2}\%$  to 25% or more.

My invention contemplates the use of a large number of buffering agents. No particular group of compounds can be specified, it being only necessary for the buffering agents to satisfy certain requirements depending on the manner of use. For example, where the buffering agent may come into contact with the sensitive emulsion, it must be one that does not affect the sensitivity of the emulsion, either by desensitization or by hypersensitization. Another requirement of the buffering agent when used in films designed to transmit light is that it should be colorless.

Among the buffering agents which I may use are oxalic, tartaric, succinic, citric, maleic, cyanuric, salicylic, and diethyl barbituric acids. Boric acid may also be used in certain concentrations. These are titrated to the proper pH by means of sodium hydroxide or some other suitable base.

It is to be understood that I am not limited in the examples given in the above specification but that my invention comprehends all modifications and equivalents coming within the scope of the appended claims.

What I claim as new and desire to secure by Letters Patent of the United States is:

1. A photographic element comprising a support, a sensitive emulsion layer on said support, and a layer containing materials capable of producing a hydrogen ion concentration different from that of the emulsion, said last mentioned layer being buffered to a hydrogen ion concentration approximately the same as that of the emulsion.

2. A photographic element comprising a support, a sensitive emulsion layer on said support, and an intermediate layer between said support and said emulsion layer, said intermediate layer being buffered to a hydrogen ion concentration approximately the same as that of the emulsion.

3. A photographic element comprising a support, a sensitive gelatin emulsion layer on said support, and an intermediate layer between said support and said emulsion layer, said intermediate layer being buffered to a hydrogen ion concentration approximately the same as that of the emulsion.

4. A photographic element comprising a transparent support, a sensitive emulsion layer on said support, and a gelatin layer between said support and said emulsion layer, said gelatin

layer being buffered to a hydrogen ion concentration approximately the same as that of the emulsion.

5. A photographic element comprising a support, a sensitive emulsion layer on one side of said support, and a layer on the opposite side of said support, said last-mentioned layer being buffered to a hydrogen ion concentration approximately the same as that of the emulsion.

6. A photographic stripping film comprising a temporary support, and as successive layers thereon, an adhesive layer, a water-permeable layer, and an emulsion layer, the adhesive layer being buffered to substantially the same hydrogen ion concentration as the emulsion layer.

7. A photographic stripping film comprising a temporary support, and as successive layers thereon, an adhesive layer, a water-permeable layer, and a gelatin emulsion layer, the adhesive layer being buffered to substantially the same hydrogen ion concentration as the emulsion layer.

8. A photographic stripping film comprising a temporary support, and as successive layers thereon, a glue-containing adhesive layer, a water-permeable layer, and an emulsion layer, the adhesive layer being buffered to substantially the same hydrogen ion concentration as the emulsion layer.

9. A photographic stripping film comprising a temporary support, and as successive layers thereon, a glue and dextrin adhesive layer, a water-permeable layer, and an emulsion layer, the adhesive layer being buffered to substantially the same hydrogen ion concentration as the emulsion layer.

10. A photographic stripping film comprising a temporary support, and as successive layers thereon, an adhesive layer, a water-permeable cellulose nitrate layer, and an emulsion layer, the adhesive layer being buffered to substantially the same hydrogen ion concentration as the emulsion layer.

11. A photographic stripping film comprising a temporary support, and as successive layers thereon, a glue-containing adhesive layer, a water-permeable cellulose nitrate layer, and an emulsion layer, the adhesive layer being buffered to substantially the same hydrogen ion concentration as the emulsion layer.

12. A photographic stripping film comprising a temporary support, and as successive layers thereon, an adhesive layer, a water-permeable cellulose nitrate layer, and a sensitive emulsion layer, the adhesive layer being buffered to substantially the same hydrogen ion concentration as the emulsion layer.

GALE F. NADEAU.